

Sept. 17, 1963

L. V. McMACKIN  
CONTINUOUS PEROXIDE BLEACHING OF CROSS  
LINKED CELLULOSE FABRICS

3,104,152

Filed Aug. 30, 1961

3 Sheets-Sheet 1



Fig. 1A

INVENTOR.

*Luther V. McMackin*  
BY

*Warley L. Parrott*

Sept. 17, 1963

L. V. McMACKIN  
CONTINUOUS PEROXIDE BLEACHING OF CROSS  
LINKED CELLULOSE FABRICS

3,104,152

Filed Aug. 30, 1961

3 Sheets-Sheet 2



Fig. 1B

INVENTOR.  
Luther V. McMackin  
BY  
Warley L. Parrott

Sept. 17, 1963

L. V. McMACKIN

3,104,152

CONTINUOUS PEROXIDE BLEACHING OF CROSS  
LINKED CELLULOSE FABRICS

Filed Aug. 30, 1961

3 Sheets-Sheet 3



INVENTOR.  
*Luther V. McMackin*  
BY  
*Warby L. Parrott*

## 1

3,104,152

## CONTINUOUS PEROXIDE BLEACHING OF CROSS LINKED CELLULOSE FABRICS

Luther V. McMackin, Lancaster, S.C., assignor to The Springs Cotton Mills, a corporation of South Carolina  
Filed Aug. 30, 1961, Ser. No. 134,980  
3 Claims. (Cl. 8—111)

The present invention relates to wash and wear fabric, and more particularly to a method for obtaining improved cellulosic wash and wear bleached fabric, in which the cellulose molecules have been cross linked by a chemical reactant.

There are two general methods for obtaining wash and wear finishes on textile fabrics. The first of these is the application of resins to the surface of a pre-bleached textile fabric, and in which discoloration does not result and subsequent bleaching is not required.

The second method for obtaining wash and wear finishes is one in which pre-bleached cellulosic fabric is reacted with a chemical that cross links the cellulose molecules. This process presents an important problem in that the cellulosic fabric is discolored by the chemical reaction, and thus subsequent bleaching is required.

Several attempts have been made to bleach fabrics having chemically cross linked cellulose molecules, such as conventional wet bleaching, boiling in bleach, and padding cold bleach onto the fabric and holding it in rolled form for a period of time, but all of the methods have disadvantages, such as being too slow for commercial purposes, damaging the wash and wear finish, and providing too low a degree of whiteness.

We have discovered a very satisfactory procedure for bleaching cellulosic fabrics to which have been imparted a wash and wear (wrinkle resistant) finish by chemically cross linking the cellulose molecules. We have found that such fabrics may be bleached with hydrogen peroxide in open width in a continuous process on hot cans, such as are most commonly used for drying fabrics, and that this overcomes the problems of insufficient speed and damage to the wash and wear finished fabric.

We have also discovered that the efficiency of the peroxide bleaching and the ultimate whiteness of the wash and wear fabric are substantially improved by carrying out the treatment of the fabric in two consecutive stages. In the first stage, the fabric is saturated with a bleaching composition containing hydrogen peroxide, and is then heated to substantial dryness, i.e. to a moisture content of about 2%—3% of the weight of the fabric. The thus treated fabric is then wet with an aqueous solution following which the fabric is heated again to substantial dryness. This procedure markedly improves the efficacy of the hydrogen peroxide and the bleaching of the fabric to desired whiteness, suitable for use in men's white shirts, etc.

An illustrative but nonlimiting embodiment of the process of this invention is shown in the accompanying drawings, in which:

FIG. 1a is a flow chart showing the first stage of the fabric treatment;

FIG. 1b is a continuation of the flow chart of FIG. 1a showing the second stage of the fabric treatment; and

FIG. 2 is a diagrammatic view of a portion of a bleaching range illustrating generally the equipment used in the two stage operation of the present invention.

According to the process of the present invention, open width, pre-bleached, woven, white, dry, cotton shirting is passed continuously at a speed of 90 yards per minute through guide rolls and into a pad box containing the following composition at 100° F., for imparting wash and

## 2

wear effects, all parts by weight, and which may be compounded by mixing together the following components, in the order listed:

|                                                                           | Lbs. |
|---------------------------------------------------------------------------|------|
| 5 39% 2,2'-sulfonyldiethanol in water                                     | 720  |
| Soda ash (99% Na <sub>2</sub> CO <sub>3</sub> )                           | 55   |
| Borax (Na <sub>2</sub> B <sub>4</sub> O <sub>7</sub> ·10H <sub>2</sub> O) | 7    |
| 25% polyethylene in aqueous dispersion                                    | 70   |
| 10 Wetting agent (1,1,3,3 tetramethylbutyl - phenoxy- polyethoxyethanol)  | 5    |

The shirting is then passed through squeeze rolls adjusted to allow the fabric to retain about 65%—70% of its own weight of the sulfonyldiethanol composition and then passed by means of a clip tenter frame for 90 feet through an area of blown hot air at 225° F. to 265° F., whereby the fabric is dried to about 5% moisture content, and then passed over a three roll calender.

The fabric is then passed through a gas fired curing oven continuously containing 150 yards of fabric and heated to 355° F. The curing temperature is critical in that below 345° F. the sulfonyldiethanol will not react with the cotton shirting to cross link the cellulose molecules, and at temperatures of more than 365° F. a cross shading of the fabric occurs that cannot be removed by subsequent bleaching. The fabric is then passed over three cooling cans, through which are circulated water at tap temperature, and then collected on a take up roll, at which time it may be stored indefinitely or taken immediately to the bleaching operation. It will be noted that the previously white cotton shirting is discolored to a cream color upon emergence from the curing oven, and that it is the thus discolored fabric that has proven so difficult to bleach.

All of the above operations have been carried out in a continuous process with the fabric traveling at a rate of 90 yards per minute.

The cotton shirting is next put through a scouring operation prior to the bleaching. We have found that the scouring is important for satisfactory subsequent bleaching. The scouring is accomplished by passing the fabric in open width continuously at a speed of 150 yards per minute over guide means and into a pad box containing, at 165° F., one gallon of concentrated acetic acid (84%), 10 pounds of detergent (33% aqueous dispersion of sodium-N-methyl-N-oleoyl laurate), and water to bring the final volume to 250 gallons, and then through squeeze rolls and into five successive wash boxes, each equipped with squeeze rolls at its entry and exit and containing 250 gallons of water at 165° F. The exit squeeze roll of the last box is adjusted to allow the fabric to retain about 50% of its weight in water. The fabric passes out onto a conventional scray to interrupt the tension.

The fabric 10 is then passed over guide means 11—13 and, while still retaining about 50% water, into a pad box 14 containing the aqueous bleaching composition. The bleaching composition is maintained at 100° F. and is continuously fed chemicals so that it has the following constant composition:

|                                                                    | Lbs. |
|--------------------------------------------------------------------|------|
| 60 50% hydrogen peroxide in water                                  | 62   |
| Wetting agent (1,1,3,3 tetramethylbutyl-phenoxy-polyethoxyethanol) | 1    |
| Soda ash (99% Na <sub>2</sub> CO <sub>3</sub> )                    | 3    |
| Sodium tripolyphosphate                                            | 50   |
| 65 Q.s. H <sub>2</sub> O to give 250 gallons final volume.         |      |

The fabric is passed through squeeze rolls 15 adjusted to allow it to emerge from the aqueous bleaching solution with about 36% of its own weight of water and aqueous bleaching solution. The fabric 10 is next passed over guides 16 and 17 and over a conventional adjustable tension device 18, and is then serpentine through a net-

work of twenty three conventional steam heated, cylindrical, rotating drying cans 19-41 in contact with the surfaces thereof. Each drying can is 72.3" in circumference and is maintained at 45 pounds per square inch internal steam pressure. The fabric remains on the above drying cans 19-41 for about 15 seconds, where the fabric is partially bleached, but not to the degree of whiteness desired. The fabric 10a emerges from drying can 41 containing about 2%-3% of its weight in residual bleach and water, about 90%-94% of the moisture content prior to can drying having been driven off of the fabric, and at which moisture content rapid bleaching has ceased for all practical purposes.

The bleaching treatment is then renewed by passing the fabric 10a into a trough 42 containing water 43 at tap temperature. This rewetting renews the action of the hydrogen peroxide and the wetted fabric then passes through squeeze rolls 44 adjusted to allow about 35% water and residual bleach retention based on the weight of the goods. While some of the bleaching composition may be removed from the fabric during the rewetting step, enough residual bleach remains on the fabric to provide the essential subsequent bleaching. The fabric 10b is passed over a series of expanders 45, and is then serpentine through a network of twenty one steam heated, cylindrical, rotating drying cans 46-66, in contact with the surfaces thereof. Each drying can is 72.3" in circumference and is maintained at 45 pounds per square inch internal steam pressure. The fabric remains on the drying cans 46-66 for about 13-14 seconds and emerges from drying can 66 substantially dry and in fully and evenly bleached bright white condition. The fabric is passed over three cooling cans 67-69, each of which is 72.3" in circumference and contains therein circulating water at tap temperature. The fabric is collected on a take up roll, and may be taken immediately into a scouring and top finishing operation or may be stored for a period of time if convenience dictates. In any event it is desirable to wash residual chemicals from the fabric to prevent damage, but we have allowed the rolled fabric with residual chemicals to stand for as long as 36 hours without damage. It will be understood that the above collection on a take up roll may be omitted if the equipment is arranged to allow the fabric to pass directly into a scouring operation, such as follows.

The fabric is next scoured by passing it continuously in open width, at the rate of 150 yards per minute, over guide means and into a pad box containing, at 165° F., one gallon of concentrated acetic acid (84%), 10 pounds of detergent (33% aqueous dispersion of sodium-N-methyl-N-oleoyl laurate), and water to bring the final volume to 250 gallons, and then through squeeze rolls and into five successive wash boxes, each equipped with squeeze rolls at its entry and exit, and containing water at 165° F.

The fabric is then dried to substantial dryness by passing it over twenty conventional steam heated, cylindrical, rotating, drying cans, in the above described manner, each being 72.3" in circumference and having an internal steam pressure of 4 lbs.-10 lbs. per square inch.

The dry fabric is passed over guide means and into a pad containing a top softener and fluorescent brightener composition at 110° F. The composition may be formed by mixing together the following components in the order listed:

25% aqueous dispersion of polyethylene \_\_\_\_ lbs. 120  
 Blue tint ("Indanthrene Blue GP Powder Fine," New  
 Color Index No. Vat Blue 4) \_\_\_\_ av. oz. 5  
 Fluorescent brightener (25% aqueous dispersion of  
 bis(2 - anilino - para - sodium sulphonate - 4 -  
 monoethanolamino - 6 - triazinyl) - 4,4' - diamino -  
 stilbene-2,2'-disodium sulphonate) \_\_\_\_ fl. oz. 30

4  
 Non-ionic wetting agent (sodium dicaprylsulfosuccinate) \_\_\_\_ lbs. 10  
 Q.s. H<sub>2</sub>O to give final volume of 250 gallons.

5 The fabric is passed through squeeze rolls adjusted to allow the fabric to retain 65%-70% of its own weight of the top softener and fluorescent brightener composition. The fabric is next dried to 5% moisture content by passing it on a clip tenter frame under a zone of hot air at 250° F. to 300° F., and finally the fabric with 5% moisture content is passed through a compressive shrinkage machine equipped with a rubber belt.

10 It will be noted that the fabric, after being collected from the curing oven, has been processed while traveling at a rate of 150 yards per minute.

15 The cotton shirting produced according to the above process has outstanding bright whiteness, excellent crease resistance in both the wet and dry states, is free from odor, and will shrink less than 0.75%. The wash and wear finish is permanent since the sulfonyldiethanol has reacted chemically to cross link the cellulose molecules.

20 I claim:

25 1. In the method of obtaining a white wash and wear cellulosic fabric wherein the cellulose is cross linked by a chemical reactant and the fabric is thereafter bleached, the improvement characterized in that the bleaching is a continuous open width process comprising the steps of impregnating a cross linked and subsequently scoured cellulosic fabric, containing about 50% of its weight in water, with an alkaline aqueous hydrogen peroxide bleaching composition containing about 3% by weight of 50% hydrogen peroxide; squeezing the fabric until it contains about 36% of its weight in water and bleaching composition; passing the fabric over and in contact with a network of heated cylindrical drying cans for about 15 seconds whereby the fabric is dried to about 2-3% of its weight in water and residual bleaching composition and partially bleached; impregnating the fabric with water; squeezing the fabric until it contains about 35% of its weight in water and residual bleaching composition; passing the fabric over and in contact with a network of heated cylindrical drying cans for about 13-14 seconds whereby the fabric is bleached to a bright white condition and substantially dried; and thereafter scouring and drying said fabric.

30 2. The method according to claim 1 and further characterized in that the cellulose is cross linked with 2,2'-sulfonyldiethanol.

35 3. The method according to claim 1 and further characterized in that said alkaline aqueous hydrogen peroxide bleaching composition comprises hydrogen peroxide, wetting agent, soda ash, and sodium tripolyphosphate.

40 55 References Cited in the file of this patent

UNITED STATES PATENTS

|           |               |               |
|-----------|---------------|---------------|
| 2,267,276 | Hager         | Dec. 23, 1941 |
| 2,858,183 | Potter        | Oct. 28, 1958 |
| 2,972,611 | Zweidler      | Feb. 21, 1961 |
| 2,983,568 | Nerney et al. | May 9, 1961   |
| 3,026,166 | Gallagher     | Mar. 20, 1962 |

FOREIGN PATENTS

|           |        |               |
|-----------|--------|---------------|
| 1,227,817 | France | June 19, 1959 |
|-----------|--------|---------------|

OTHER REFERENCES

Dorest: "The Textile Manufacturer," May 1954, page 254.

70 Andrews et al.: Textile Research J., vol. 32, No. 6, June 1962, pages 489-496.

Ward Chemistry and Chemical Technology of Cotton, pages 507-509, pub. 1955 by Interscience Publishers Inc., New York. (TS-1542W2 C. 2 and Div. 43.)